

## CORROSION INHIBITION COMPOSITIONS

Glenn A. Marsh and Edward Schaschl, Crystal Lake, Ill., assignors to The Pure Oil Company, Chicago, Ill., a corporation of Ohio

No Drawing. Filed Dec. 6, 1956, Ser. No. 626,605.

15 Claims. (Cl. 252—389)

This invention relates to a method of preventing the corrosion of ferrous metals by aqueous ammonia-ammonium nitrate environments. More particularly, the invention relates to a stable, substantially thixotropic corrosion-inhibiting composition containing 2-mercaptopbenzothiazole as the principal active ingredient along with certain prescribed proportions of a metal nitrite and an oxidizing agent which are chemically inert to the mercaptobenzothiazole in an aqueous gel composition. This application is a continuation-in-part of the application entitled, Corrosion Inhibition in Aqueous Ammonia-Ammonium Nitrate Systems, filed October 10, 1955, by Glenn A. Marsh and Edward Schaschl and bearing Serial Number 539,690, now abandoned.

In accordance with the aforesaid copending application, it is shown that environments containing ammonia-ammonium nitrate in an aqueous medium are utilized as liquid fertilizers on a commercial scale. Such fertilizer solutions present a severe corrosion problem in the apparatus used in the preparation, storing, handling, and dispensing of same. Ferrous metal processing equipment as well as the tank cars, other types of metallic shipping containers, and dispensing apparatus for use in the field are subjected to very rapid corrosion by these fertilizer solutions, far exceeding that encountered when the ferrous metal is in contact with an ordinary aqueous environment. A particularly severe corrosion problem is evidenced where part of the ferrous metal is in contact with the corrosive fertilizer liquid and a part of the ferrous metal is exposed to an oxygen-containing environment, such as exists when a ferrous metal tank is only partially filled with the fertilizer solution and has an air space above the liquid level. When dissolved oxygen is present in substantial amounts, that is more than about 0.1 p.p.m., the corrosion problem is accentuated.

Another instance in which the inhibition of corrosion of ferrous metal is particularly difficult occurs when a metal surface has undergone exposure to certain agents, such as by contact or association with a more active metal, for example a steel container, zinc, or other active metal, or by contact with an abrasive or by dipping the ferrous metal into a strong acid such as hydrochloric acid of any suitable concentration before exposure to the corrosive environment. The present invention has three main purposes: First, that of providing a convenient means for bringing mercaptobenzothiazole into a corrosive environment of the general type aforementioned for the purpose of mitigating the corrosion. A second purpose of the invention is to provide a substantially thixotropic corrosion inhibitor composition containing the mercaptobenzothiazole, a metal nitrite and an oxidizing agent in an aqueous medium, in which form the composition is easy to produce, stable and exhibits good corrosion-inhibiting properties. The third purpose of the invention is to provide a corrosion-inhibiting composition containing mercaptobenzothiazole which is in a form that is convenient for handling and packaging and also convenient for use in

the field. These primary purposes apply whether the composition is used for the general corrosion-inhibiting properties of mercaptobenzothiazole in an ammonia-ammonium nitrate corrosive environment, or used to overcome corrosion under conditions of aeration or activation of the metal surface, which conditions having just been described. For the purpose of this invention, therefore, when the corrosive solution contains less than about 0.1 p.p.m. of oxygen, it is said to be deaerated and when it contains more than about 0.1 p.p.m. of oxygen it is said to be aerated. Likewise, for purposes of this invention, the metal surface is said to be "activated" when a condition is imposed which renders the metal more easily corrodible in the presence of oxygen, as by a galvanic effect or acid etching.

Heretofore many inhibitors have been proposed for retarding the corrosion of ferrous metals in aqueous environments. Inhibitors placed in ammonia-ammonium nitrate solutions retard corrosion only in the liquid and have no effect upon corrosion which occurs above the liquid level. The particular fertilizer solutions with which this invention is concerned, comprising as they do ammonia and ammonium nitrate in aqueous solution, afford a unique corrosive environment, particularly when substantial concentrations of these ingredients are present, such as fertilizer containing a concentration of approximately 10% or more of nitrogen by weight. The stability, physical form and effectiveness of the inhibitor compositions of this invention for aqueous systems in an ammonia-aqueous ammonium nitrate environment cannot be predicted.

In accordance with this invention, it has been found that a stable, substantially thixotropic corrosion-inhibiting composition which is capable of being pumped can be made by thoroughly agitating between about 15 to 30 weight percent of finely divided mercaptobenzothiazole as the solid phase in a liquid phase comprising water. The exact percentage of mercaptobenzothiazole that will form a stable suspension in an aqueous medium depends somewhat on the time, the rate of stirring, and the particle size of the mercaptobenzothiazole. However, by using the powdered form of mercaptobenzothiazole which is commercially available, a stable substantially thixotropic suspension can be formed by thorough mixing of about 18 to 27% by weight of mercaptobenzothiazole with water.

In accordance with the aforesaid parent application, the disclosure of which is incorporated by reference, the presence of certain limited amounts of a metal nitrite and an oxidizing agent enhance the corrosion inhibiting properties of the mercaptobenzothiazole. Now in accordance with this invention, as another aspect thereof, it has been found that the inclusion of these auxiliary nitrites and oxidizing agents, to be described, does not prevent the formation of a stable substantially thixotropic, fixed composition suspension, of from 15 to 46 weight percent of mercaptobenzothiazole in water or aqueous suspensions containing up to 20 wt. percent of an anti-freeze agent.

Furthermore, it has been found that there is a certain essentially critical relationship between the ratio of solids to total liquids in the suspension and the weight of anti-freeze agent present. These nitrites and oxidizing agents can be dissolved in the water phase either before or after the mercaptobenzothiazole is added and are carried in solution to the limit of their solubilities in the liquid phase. The mercaptobenzothiazole forms the solid suspended phase. The preferred corrosion-inhibitor compositions of this invention contain about 15 to 30 weight percent of mercaptobenzothiazole suspended in sufficient water to make 100% and also include (1) such suspensions containing a metal nitrite in an amount of about

0.25 to 2.5 times the amount of mercaptobenzothiazole and an amount of an oxidizing agent, particularly sodium or potassium chlorate, in an amount of about 0.05 to 0.2 times the amount of mercaptobenzothiazole, and (2) such suspensions containing from 15 to 46% solid phase with or without the nitrite and oxidizing agent, containing up to 20% by weight of an anti-freeze agent.

A first object of this invention is to provide a new and useful physical form of a corrosion-inhibitor composition containing mercaptobenzothiazole, in an aqueous suspension with or without a metal nitrite, an oxidizing agent and an anti-freeze agent.

A further object of this invention is to provide a corrosion-inhibiting composition containing mercaptobenzothiazole, for use in inhibiting the corrosivity of ammonium-ammonium nitrate environments, which is of a substantially thixotropic character and has a semi-solid consistency, but which is, upon the application of agitation or shear, transformed into a mobile fluid for easy handling and dispensing.

Other objects of this invention will be apparent or set forth in the following detailed description.

The invention may be illustrated by the following specific examples.

#### EXAMPLE 1

100 parts by weight of dry inhibitor consisting of a mixture of 77 parts of powdered mercaptobenzothiazole, 19.2 parts of sodium nitrite, and 3.8 parts of potassium chlorate were stirred with 372 parts of water at room temperature. There resulted a suspension comprising about 78% water and about 22% solids which exhibited thixotropic properties and had a semi-solid consistency similar to that of thick cream or a grease. Upon standing, the composition formed into a fairly firm gel. However, by stirring the sample with a stirring rod the gel structure was easily broken and the composition became liquid in form. Upon termination of agitation the gel structure formed again. Several separate preparations were carried out in the aforementioned manner with the same results illustrating the reproducibility of the stable suspension.

#### EXAMPLE 2

A portion of the gel composition from Example 1 was thoroughly agitated with about 10 parts by weight of water. It was found that the gel dispersed in the water, but within a matter of hours it reverted to its original form as a separate layer under the additional added water. This illustrates the stability of the composition.

#### EXAMPLE 3

The gradual addition of incremental amounts of powdered mercaptobenzothiazole alone to 400 grams of water with constant agitation produced a heavy, stable suspension having the consistency of cream when about 120 grams or 23% by weight of mercaptobenzothiazole had been added. This material was transformed into a mobile liquid by the shearing action of a stirrer or pump.

It has been found that a substantial part of the water in the aforesaid compositions may be replaced with an anti-freeze material such as alcohol, glycerine and the various glycols, including ethylene glycol, without disturbing the thixotropic characteristics thereof. The anti-freeze agent allows the percentage of solids to be increased in a certain relationship to the amount of the anti-freeze added. Methanol and ethanol or mixtures of same may be used as anti-freeze agents. This weight ratio is expressed as follows:

$$S = 2.85A + 0.28$$

where  $S$  is the ratio of solids to total liquids, and  $A$  is the weight fraction of alcohol or other anti-freeze agent. This relationship holds for anti-freeze concentrations up to about 20% which is also the upper limit necessary to provide adequate protection of the composition against

freezing in a temperate zone. Thus, at an anti-freeze concentration of 20%,  $A$  will be 0.2; and hence

$$S = 2.85(0.2) + 0.28$$

5 or is equal to 0.85. Also,  $S$  equals the weight of total solids per gram of mixture divided by 0.2 (the weight fraction of anti-freeze) plus the weight of water. The weight of solids plus the weight of water plus the weight of anti-freeze = 1.0. By solving these equations the percentage of solids = 46%, the percentage of water = 34% and the percentage of anti-freeze = 20%. It is thus seen that by incorporating an anti-freeze agent in the composition to the extent of about 20% the total solids can be increased from about 22% to about 46%.

15 This is demonstrated by the following experiments.

#### EXAMPLE 4

20 400 grams of a dry inhibitor mixture containing 77% 2-mercaptobenzothiazole, 19.2% sodium nitrite and 3.8% potassium chlorate were mixed with incremental amounts of water and Formula 30 alcohol (81.12% by weight ethyl alcohol and 18.88% by weight of methyl alcohol) and after each mixing the solids-liquid mixture was allowed to stand. This procedure was repeated, each 25 time adding more measured quantities of water and alcohol and observing the results after thorough shaking of the mixture until a stable, thixotropic mixture was obtained. This occurred when 400 grams of water and 150 grams of alcohol had been added. On a weight percent basis this composition contained about 32.4% mercaptobenzothiazole, 8.1% sodium nitrite, 1.6% potassium chlorate, 42.1% water and 15.8% alcohol.

#### EXAMPLE 5

30 35 100 grams of a dry inhibitor mixture containing 77% 2-mercaptobenzothiazole, 19.2% sodium nitrite and 3.8% potassium chlorate were mixed with incremental amounts of water alone and after each mixing the solids-liquid mixture was allowed to stand. When 370 grams of water 40 had been added a thixotropic mixture resulted. On a weight percent basis this composition contained 16.38% mercaptobenzothiazole, 4.08% sodium nitrite, 0.81% potassium chlorate and 78.73% water.

45 By substituting the data obtained in Examples 3 and 4 into the general equation for a straight line, which is

$$y = ax + b$$

50 the values of  $a$  and  $b$  were determined to be 2.85 and 0.28, respectively, where  $y$  is the ratio of solids to total liquid and  $x$  is the weight fraction of alcohol in the total mixture. Replacing  $y$  by  $S$  and  $x$  by  $A$  the equation referred to results.

55 The applicability of this equation was checked by calculating the theoretical composition of a thixotropic mixture containing 20% by weight of alcohol. It was calculated that a mixture of 46% solids, 34% water and 20% alcohol should be thixotropic. This was substantiated by mixing together 460 grams of the solid inhibitor mixture with 340 grams of water and 200 grams 60 of alcohol, which mixture exhibited thixotropic properties. Furthermore, the addition of more water to the mixture did not destroy these properties.

65 The method of utilizing the thixotropic mixture of this invention does not depart from the method of use described in the aforementioned co-pending continuation-in-part application, Serial Number 539,690. The thixotropic mixture is added directly to the corrosive aqueous ammonium nitrate-ammonia solution in any suitable manner, that is, all at once, or in small or large increments, or continuously, with or without agitation of the resulting homogeneous solution. The fact that the corrosion-inhibiting composition is in a mixed thixotropic semi-liquid form does not change the minimum requirements of active ingredients necessary to inhibit corrosion. The amount of the thixotropic mixture used is suffi-

cient to maintain or add a minimum of about 0.01% by weight of 2-mercaptopbenzothiazole, and preferably about 0.1% by weight based on the weight of total solution. Accordingly, it is seen that very small amounts of the active ingredients of the thixotropic mixture may be used to obtain effective results. The addition of the inhibitor composition to the aqueous fertilizer solution in no way effects its utility or ease of handling. The resulting blend is homogeneous and essentially colorless, although the thixotropic mixture of the inhibitor composition itself is a yellow color due to the mercaptobenzothiazole. If desired, the yellow color can be changed to a faint orange by the addition of small amounts, 0.1 to 2.0 percent by weight, of a red azo-dye, such as Congo red. The use of larger amounts of dye may destroy the suspension, so if it is desired to color the composition, the effect of any contemplated dye must be determined by mixing experimental batches.

The addition of the corrosion inhibiting composition to the aqueous ammonium nitrate-ammonia fertilizer solutions inhibits the corrosion of ferrous metals which are totally immersed therein and which are partially exposed to an oxygen-free atmosphere where the oxygen is absent from the solution if the metal has been activated as before described. The composition of this invention is also effective in inhibiting the corrosion of totally immersed activated ferrous metals where dissolved oxygen is present, or of activated metals in contact with both an oxygen-containing ammonium nitrate-ammonia solution and with a non-oxygen-containing atmosphere, because of the inclusion of the nitrite and the inorganic oxidizing agent. In addition to the sodium nitrite previously mentioned, other metal nitrates soluble in the corrosive solution may be used, such as potassium nitrite, lithium nitrite, cesium nitrite and barium nitrite. The solid inorganic oxidizing agent, chemically inert to the other components of the combination inhibitor and soluble in the corrosive solution, may include any alkali metal chromate such as sodium chromate, or any alkali metal chlorate such as potassium chlorate. Ammonium chromate, sodium chlorate or potassium chromate may be used. Where 15 parts of 2-mercaptopbenzothiazole are used with 85 parts of water, with or without sufficient antifreeze to prevent freezing of the mixture during winter months, the amount of nitrite present may be 3.75 parts and the amount of oxidizing agent present may be .75 part. Where 30 parts of 2-mercaptopbenzothiazole are used with 70 parts of water with or without sufficient antifreeze to prevent freezing of the mixture during winter months, the amount of nitrite present may be 75 parts and the amount of oxidizing agent may be 6.0 parts. In this way between about 0.1 to 0.5 wt. percent of nitrite and 0.01 to 0.5% of oxidizing agent are incorporated in the corrosive ammonium nitrate-ammonia fertilizer solution. Preferably the concentration of the nitrite is between about 0.2 and 0.5% and the oxidizing agent between about 0.01 and 0.5 wt. percent in the corrosive atmosphere. A minimum concentration of the combination inhibitor of about 0.12% by weight based on the corrosive solution should be used, as described and developed in the parent application, Serial Number 539,690, to effectively and substantially completely inhibit the corrosion of totally immersed ferrous metals contacted by the corrosive fertilizer solutions in the presence or absence of dissolved oxygen in the corrosive solution.

The ferrous metal-containing apparatus to be protected from the corrosive solution may be of any shape or size, such as storage tank, a tank carrier, flow pipe, conveying coil, measuring tank or any type of processing apparatus such as a mixing tank, settling tank, ammoniation tank, etc., and is constructed of metal or alloy, containing an appreciable amount of iron, such as cast iron, wrought iron or low carbon steel. As stated above, the metal to be protected may be in an unactivated or activated state.

To insure complete protection when the ferrous metal or alloy is exposed not only to the liquid corrosive solution but also to an oxygen-containing gaseous phase adjacent the corrosive solution, additional protection must be afforded the metal or alloy to prevent corrosion of that portion exposed to the gaseous phase. This is accomplished by adding a blanket of a chemically inert liquid which is immiscible with the corrosive solution and lighter in gravity. This inert liquid may be any material which is liquid under existing conditions, is essentially immiscible and nonreactive with the corrosive solution and is lighter in gravity than the corrosive solution containing the inhibitor mixture of this invention. Examples are liquified propane, naphtha such as rubber solvent, textile spirits, V.M. and P. naphtha, Stoddard solvent, kerosene, fuel oils of any viscosity and of a petroleum origin, prepared in any conventional manner, such as by fractionation, gas oils of a petroleum-derived nature and prepared in any conventional manner, neutral lubricating oils, and highly refined lubricating oil fractions, such as white oil. Aliphatic and/or alicyclic hydrocarbon-containing oils are preferred and aromatic oils should not be used.

The blanketing immiscible liquid is added to the corrosive solution in a sufficient concentration to embody a surfactant and also completely extend over the surface of the corrosive solution in a layer of sufficient depth or thickness to act as an effective barrier against penetration by the atmosphere above and form a thin film on the metal wall or surface as the level of the corrosive solution rises and falls in the metal container. A layer having a thickness of  $\frac{1}{4}$  inch is sufficient for most purposes. Any oil-soluble, water-insoluble, semi-polar surfactant which renders the metallic surface hydrophobic may be used. The surfactant should be chemically inert to the other chemical compounds present in the corrosive solution and essentially non-extractable by the corrosive solution. Any suitable surfactant having the above characteristics, such as an amine salt (primary, secondary, or tertiary) or ammonium salt of a fatty acid containing more than about 12 carbon atoms, or any combination of two or more of such salts may be used. The surfactant is present in a total concentration of at least about 0.1%, by weight, of the blanketing agent. Concentrations of about 0.5 to 1.0% by weight are preferred, in general, but larger concentrations, such as 2% by weight, may be employed and may even be desirable in those instances where there may be a tendency for the particular surfactant or combination of surfactants used to be extracted to some extent by the corrosive aqueous ammonia-ammonium nitrate solution.

Although any amine salt of a fatty acid, or any combination thereof, may be used without reference to the chain length of the amine component of the salt, amines containing at least one long hydrocarbon chain above about 12 carbon atoms in length, particularly chains derived from fatty acids such as oleic, stearic, palmitic, linoleic, etc., are preferred. For example, a very satisfactory commercial product, Duomeen T dioleate, may be used in effective concentrations of about 0.1% by weight or more, preferably 0.2% by weight or more. Duomeen T dioleate is the dioleic acid salt of an organic base Duomeen T, which is a member of a group of fatty diamines. Duomeen T dioleate is a product of the Armour Chemical Division of Armour & Company.

Other suitable surfactants are ammonium oleate, stearyl amine palmitate, oleylamine ricinoleate, and stearylamine stearate. The function of the surfactant is to render the metal surface hydrophobic, reduce interfacial tensions and hinder or prevent "creeping" of the corrosion solution up on the metal surface above the liquid level. When the solution "creeps" upon the metal surface it evaporates and causes extensive corrosion, in conjunction with oxygen, and the formation of a thick crust on the metal on those wetted areas.

Handling of the gel-like suspension of this invention is

facilitated by the thixotropic properties which means that agitation, shear, vibration, or coning may be used to transform the suspension into a mobile liquid. The composition is readily handled by a slurry pump or the type of pumps used to move drilling muds. A Moyno pump has been found to be particularly adapted for this purpose.

The invention therefore comprises the discovery of a stable, substantially thixotropic form of corrosion inhibiting composition containing 2-mercaptopbenzothiazole, with or without a metal nitrite, and with or without an oxidizing agent, as the solid phase suspended in an aqueous or aqueous-anti-freeze-containing solution which is particularly easy to handle, package and use in carrying out the method of corrosion inhibition described in the parent application heretofore referred to. The following table shows the composition of eight different compositions prepared in accordance with the invention, all of which exhibit the unusual property of resisting further dilution upon being mixed with water and exhibiting thixotropic

nitrite and barium nitrite equivalent to about 0.25 to 2.5 times the amount of 2-mercaptopbenzothiazole, an amount of an oxidizing agent selected from the group of alkali metal chlorates and alkali metal chromates equivalent to about 0.05 to 0.2 times the amount of 2-mercaptopbenzothiazole and an aliphatic alcohol antifreeze agent as parts of the aqueous phase, the weight ratio of said solid phase to the total liquid phase being equal to  $2.85A + 0.28$  where A is the weight fraction of said aliphatic alcohol antifreeze agent and A has an upper limit of about 20 percent by weight based on the total composition.

5 7. The thixotropic composition in accordance to claim 6 in which the oxidizing agent is an alkali metal chromate.

8. The thixotropic composition in accordance with claim 6 in which the oxidizing agent is an alkali metal chloride.

10 9. A thixotropic composition in accordance with claim 6 in which the aliphatic alcohol antifreeze agent is ethyl alcohol.

#### THIXOTROPIC CORROSION INHIBITING COMPOSITIONS

|           | (1)   |             | (2)   |             | (3)   |             | (4)   |             | (5)    |             | (6)   |             | (7)    |             | (8)    |             |
|-----------|-------|-------------|-------|-------------|-------|-------------|-------|-------------|--------|-------------|-------|-------------|--------|-------------|--------|-------------|
|           | Parts | Wt. Percent | Parts | Wt. Percent | Parts | Wt. Percent | Parts | Wt. Percent | Parts  | Wt. Percent | Parts | Wt. Percent | Parts  | Wt. Percent | Parts  | Wt. Percent |
| Water     | 70    | 64.2        | 70    | 38.7        | 70    | 39.6        | 70    | 61.7        | 85     | 81.4        | 85    | 61.0        | 85     | 61.5        | 85     | 79.5        |
| Mercapto- |       |             |       |             |       |             |       |             |        |             |       |             |        |             |        |             |
| benzo-    | 30    | 27.5        | 30    | 16.6        | 30    | 17.0        | 30    | 26.4        | 15     | 14.8        | 15    | 10.7        | 15     | 10.9        | 15     | 14.1        |
| thiazole  |       |             |       |             |       |             |       |             |        |             |       |             |        |             |        |             |
| Metal     |       |             |       |             |       |             |       |             |        |             |       |             |        |             |        |             |
| Nitrite   | 7.5   | 6.8         | 75    | 41.4        | 75    | 42.5        | 7.5   | 6.6         | 3.75   | 3.6         | 37.5  | 26.2        | 37.5   | 26.9        | 3.75   | 3.5         |
| Oxidizing |       |             |       |             |       |             |       |             |        |             |       |             |        |             |        |             |
| Agent     | 1.5   | 1.4         | 6     | 3.3         | 1.5   | .85         | 6.0   | 5.3         | .75    | .7          | 3.0   | 2.1         | .75    | .6          | 3.0    | 2.9         |
|           | 109.0 | 99.9        | 181.0 | 100.0       | 176.5 | 99.9        | 113.5 | 100.0       | 104.50 | 100.0       | 140.5 | 100.0       | 138.25 | 99.9        | 106.75 | 100.0       |

What is claimed is:

1. A stable substantially thixotropic composition comprising a mixture of about 15 to 46 weight percent of 2-mercaptopbenzothiazole, as the solid phase suspended in a sufficient amount of an aqueous phase containing an aliphatic alcohol antifreeze agent to make 100% total composition in which the weight ratio of the solid phase to the total liquid phase is equal to  $2.85A + 0.28$  where A is a weight fraction of said aliphatic alcohol antifreeze agent and A has an upper limit of 20 percent by weight.

2. A thixotropic composition in accordance with claim 1 in which the aliphatic alcohol antifreeze agent is ethyl alcohol.

3. A thixotropic composition in accordance with claim 1 in which the aliphatic alcohol antifreeze agent is a mixture consisting of 81.12% by weight of ethyl alcohol and 18.88% by weight of methyl alcohol.

4. A thixotropic composition in accordance with claim 1 in which the aliphatic alcohol antifreeze agent is a glycol.

5. A thixotropic composition in accordance with claim 4 in which the glycol is ethylene glycol.

6. A stable substantially thixotropic corrosion inhibiting composition capable of inhibiting the corrosion of ferrous metals by solutions comprising ammonium nitrate, water and ammonia which comprises about 15 to 46 weight percent of 2-mercaptopbenzothiazole, as the solid phase suspended in a sufficient amount of water to make 100 percent by weight total composition, an amount of a metal nitrite selected from the group consisting of sodium nitrite, potassium nitrite, lithium nitrite, cesium

40 10. A thixotropic composition in accordance with claim 6 in which the aliphatic alcohol antifreeze agent is a mixture consisting of 81.18% by weight of ethyl alcohol and 18.88% by weight of methyl alcohol.

11. A thixotropic composition in accordance with claim 6 in which the aliphatic alcohol antifreeze agent is a glycol.

45 12. The thixotropic composition in accordance with claim 7 in which the alkali metal chromate is sodium chromate.

13. The thixotropic composition in accordance with claim 8 in which the alkali metal chloride is potassium chloride.

50 14. A thixotropic composition in accordance with claim 11 in which the glycol is ethylene glycol.

15. A thixotropic corrosion inhibiting composition consisting of a mixture of about 32.4% by weight of mercaptopbenzothiazole, about 8.1% by weight of sodium nitrite, about 1.6% by weight of potassium chloride, about 42.1% by weight of water and about 15% by weight of a mixture consisting of 81.12% by weight of ethyl alcohol and 18.88% by weight of methyl alcohol.

60

References Cited in the file of this patent

#### UNITED STATES PATENTS

|           |                 |                |
|-----------|-----------------|----------------|
| 2,054,282 | Clarkson et al. | Sept. 15, 1936 |
| 2,238,651 | Keenan          | Apr. 15, 1941  |
| 2,478,755 | Elder           | Aug. 9, 1949   |
| 2,692,860 | Barker          | Oct. 26, 1954  |
| 2,815,328 | Green et al.    | Dec. 3, 1957   |